

# UNITED STATES PATENT OFFICE.

JOHN GEO. PERZÉL, OF NEW YORK, N. Y.

## IMPROVED PROCESS OF RECOVERING WOOL FROM MIXED FABRICS.

Specification forming part of Letters Patent No. 39,828, dated September 8, 1863; antedated April 3, 1863.

*To all whom it may concern:*

Be it known that I, JOHN GEORGE PERZÉL, of the city, county, and State of New York, have invented a certain new and Improved Mode in Separating Wool from Cotton; and I do hereby declare that the following is a full and exact description thereof.

The nature of my invention consists in destroying the cotton in old mixed woolen goods by means of chloride of zinc or analogous chlorides, either alone or with the aid of diluted sulphuric acid, whereby the wool remains, without being injured, as a new and useful article of manufacture.

I am aware that sulphuric acid has been used to render the mentioned effect—an application which is in accordance with the well-known chemical fact that sulphuric acid has the property of dissolving or decomposing cotton, forming dextrine and sugar, &c.; but as this acid is of a very powerful chemical character, great care must be observed in using the same for the purpose mentioned. It is a matter of course that the wool cannot resist a continued action of sulphuric acid, and particularly not a raising of temperature by the presence of this powerful agent. Nevertheless this process has till yet been observed, but at the same time under a continuation of many troubles. The nature of the process and the destroying agent used explains fully why difficulties are experienced which hardly are to be avoided.

To overcome these difficulties is the object of my invention—namely, in the use of chloride of zinc or chloride of calcium or other analogous chlorides. These substances possess the same property as sulphuric acid. They destroy cotton by raising the temperature to about 100° centigrade without injuring the wool under the same circumstances. The goods may remain in this liquid substance, hereinafter described, for twenty-four hours without destroying the wool, &c. It is possible, and under some circumstances practicable, to bring the goods in concentrated boiling solution of the before-named substances for fifteen minutes, &c., and the result will be as is required. It is otherwise very easily understood why these substances are more convenient for the workmen than sulphuric acid, as it is well explained in the nature of the same why the separating and destroying process mentioned can better and with ease be controlled.

To enable others to make and use my invention, I will now proceed to describe the *modus operandi*.

I take common muriatic acid, dissolve in it as much metallic zinc as is possible, and boil it down to an oily consistency. Of this liquid I use about one hundred and fifty gallons at once, (or more under some circumstances,) and bring in it as much from the woolen goods, which are before washed in order to remove the fatty matter, in a manner as may be learned from any good book of chemical technology, (see Knapp's Hand-Book of Technology,) as may be convenient to work with, and let it remain in this state for a while—say half an hour. The goods are then taken out and wrung in order to remove the surplus liquid. This may be done in a shorter time and by saving of labor by means of a centrifugal machine. From here the goods are placed in a drying or roasting apparatus of a similar construction as the malt-roasters, &c. Samples which from time to time are taken out show when the process is to end. This will be the case when the cotton texture becomes ruined by feeble rubbing, whereby the cotton is removed in form of dust. A little practice will enable everybody to judge about the time. After this the goods must be well washed, dried, and brought in a rubbing (Walf) machine, where the destroyed cotton is separated and removed from the wool, &c. They are at last brought through different machines as they are used in woolen manufacture, in order to obtain a nice article of commerce.

In some respects—as in order to shorten the destroying process—it may be practicable to use chloride of zinc with the aid of diluted sulphuric acid. In this case it is only necessary to bring the goods, after they have passed the zinc solution, in a mixture of water and sulphuric acid of about 15° Baumé for about fifteen minutes, &c.

Having now fully described my invention, what I claim as new, and desire to secure by Letters Patent, is—

The solution of chloride of zinc or analogous chlorides, either alone or with the aid of diluted sulphuric acid, in a manner as described, and for the purpose set forth.

JOHN GEORGE PERZÉL.

Witnesses:

CHAS. F. SONNEBORN,  
FR. RUSCHHAUPT.